

## UNITED STATES PATENT OFFICE

2,019,834

PRODUCTION OF PLYWOOD AND OTHER  
JOINED WOODEN ARTICLES

Karl Vierling, Matthias Schmhing, and Hugo Klingenberg, Ludwigshafen - on - the - Rhine, Germany, assignors to I. G. Farbenindustrie Aktiengesellschaft, Frankfort - on - the - Main, Germany

No Drawing. Application July 11, 1930, Serial No. 467,384. In Germany July 24, 1929

5 Claims. (Cl. 144—309)

The present invention relates to the production of plywood and other joined wooden articles.

In the production of plywood and other joined wooden articles in which at least one thin slab of wood is combined with another wooden surface the single wooden layers are usually joined with the aid of adhesives made from common glue or from casein, the process consisting for example in painting one or more single slabs of veneer with viscous adhesive preparations, combining the coated slabs and subjecting them to high mechanical pressure, if desired while heating. When employing common glue the process is rather tedious due to the long period of time required by the glue for obtaining its maximum of adhesiveness. Preparations from casein can be applied in the form of the so-called cold glues, in contrast to common glue which is usually applied in the form of a hot viscous solution. The 10 employment of cold glues from casein is, however, met with several disadvantages and neutral solutions of condensation products from urea and formaldehyde have been suggested as substitutes for the adhesives from casein. These preparations from the said condensation products are quite satisfactory for combining paper, leather or other soft materials but for the production of plywood and other joined wooden articles these preparations have not proved entirely satisfactory.

We have now found that plywood and other joined wooden articles with a particularly high strength can be obtained when the single parts, for example slabs of veneer, are coated with a 15 solution of a water-soluble condensation product of a urea and formaldehyde to which solution a small amount of an acid reacting agent has been added shortly before coating the surfaces to be joined. By the said addition the single parts of wood are firmly joined in a short time on pressing the combined layers in a mechanical press, the quantity of acid reacting agent being usually from about 0.4 to 2 per cent by weight of the urea-formaldehyde condensation product. 20 The said upper limit should not be exceeded since otherwise the glue may be rendered too viscous for easily coating the slabs and solidifies too quickly. The said acid reacting agents may be chosen from acids such as hydrochloric, sulphuric, phosphoric, acetic, oxalic, lactic acids, acid reacting salts such as acid sodium sulphate, mono-ammonium phosphate or aluminium chloride, and agents which split off acids when incorporated with the mixture, such as ammonium chloride, ammonium sulphate, copper sulphate or copper

chloride. In order to improve the uniform dispersion of the glue onto the wood and the desired degree of viscosity, starch, potato flour, ground potato flakes or other pulverized fillers of most different nature may be added.

The aforesaid water-soluble condensation products from urea and formaldehyde may be obtained for example by condensing a urea and formaldehyde in the presence of water and/or of an organic solvent with the aid of an acid 10 condensing agent, such as the acid agents mentioned above or the so-called buffer compounds or buffer mixtures as for example monosodium phosphate or a mixture thereof with di-sodium phosphate, or the urea and formaldehyde may be 15 first condensed in the presence of a small quantity of alkali whereby methylol derivatives of the urea employed are formed and these methylol compounds, such as mono- or di-methylol urea, mono- or di-methylothiourea and the like, may 20 be then further condensed with the aid of acid condensing agents; care being taken, however, that the condensation is not carried so far that water-insoluble products are obtained. When 25 the condensation has been carried out in the presence of such quantities of water that the condensation products are obtained in the form of their aqueous solutions of such concentration that they may be directly employed for the purpose of the present invention, no dilution with water 30 or, on the other hand, evaporation of water will be required, the strength of the solutions employed for the present process being usually between 20 and 50 per cent of condensation product 35 of the solutions. These solutions usually possess a rather low viscosity, especially those with a low content of condensation products and their viscosity may be easily increased by the before-mentioned addition of carbohydrates or flour, which are usually employed in quantities of from 40 5 to 40 per cent by weight of the solutions and do not impair the adhesive power of the glue. If desired up to 10 per cent of an animal glue such as common bone-glue or casein may be added.

The plywood and other joined wooden articles obtained in the aforesaid manner show a particularly high strength which is higher than that of joining with the aid of glue from a urea-formaldehyde condensation product free from acid reacting agent, the joints being moreover highly 50 resistant to water. In any case the single original parts of wood cannot be torn off from each other as such along the joint but the wood breaks within the fibres.

The following examples will further illustrate 55

how the present process may be carried out in practice but the invention is not restricted thereto.

*Example 1*

5      200 kilograms of 30 per cent aqueous formaldehyde are incorporated with 100 grams of mono-sodium phosphate and heated to 95° C. A solution, heated to 70° C., of 60 kilograms of urea in  
 10     30 kilograms of water is then introduced into the solution of formaldehyde and 150 grams of tri-sodium phosphate are added whereupon the mixture is evaporated in vacuo and below 50° C. until it has a content of 35 per cent of condensation  
 15     product.  
 1000 parts of the 35 per cent aqueous solution are stirred with 200 parts of potato starch, whereupon 10 parts of 2 N-sulphuric acid are added. The glue obtained remains in the liquid condition  
 20     for from 8 to 12 hours within which time slabs of beech wood of 1.5 millimetres thickness are coated with the preparation and then the whole is pressed for 5 minutes at 100° C. and at a pressure of 20 kilograms per square centimetre. When  
 25     the veneers have been joined while crossing the grain the strength of the product is from 25 to 27 kgs. per square centimetre, whereas when the slabs have been joined in parallel direction of the grain a strength of from 60 to 80 kilograms per square  
 30     centimetre is obtained.

*Example 2*

35     1000 parts of an aqueous 45 per cent solution of the condensation product prepared according to Example 1 are incorporated with 10 per cent of wheat flour and 30 parts of 5 per cent aqueous ammonium chloride. Slabs of beech wood which are 2 centimetres wide and 0.4 centimetre thick are coated with the glue and then pressed at 100°

C. for 8 minutes at a pressure of 20 kilograms per square centimetre. The strength of the finished product is from 90 to 140 kilograms per square centimetre when the slabs have been joined in parallel direction of the fibres in the single slabs, 5 whereas the strength is from 40 to 50 kilograms per square centimetre only when no ammonium chloride has been added.

What we claim is:—

1. The process of joining wooden surfaces which comprises applying to said surfaces a solution of a water soluble condensation product of a urea and formaldehyde to which condensation product an acid reacting agent inert to formaldehyde has been added shortly before the solution applying 15 step is effected and pressing the surfaces together at an elevated temperature.
2. The process according to claim 1 in which the pressure is about 20 kilograms per square centimeter and the temperature is about 100° C. 20
3. The process according to claim 1 in which the acid reacting substance is added in an amount ranging from .4 to 2 per cent of the weight of the condensation product.
4. The process according to claim 1 in which 25 the solution of condensation product employed is a water solution to which a thickening agent has been added.
5. The process of joining wooden surfaces which comprises applying to said surfaces a solution of 30 a water soluble condensation product of a urea and formaldehyde to which condensation product an acid reacting agent inert to formaldehyde has been added shortly before the solution applying step is effected and pressing the surfaces together. 35

KARL VIERLING.  
 MATTHIAS SCHMIHING.  
 HUGO KLINGENBERG.